# EUROPEAN PATENT SPECIFICATION

(11) **EP 1 141 454 B1**
(45) Date of publication and mention of the grant of the patent: **29.03.2006**
(21) Application number: 99960637.9
(22) Date of filing: 02.12.1999
(51) Int. Cl.: D01F 6/66, D01F 6/84, D01F 6/86, D01F 8/14, D01F 8/16, D04H 1/54

(54) **THERMOPLASTIC FIBERS AND FABRICS**
THERMOPLASTISCHE FASERN UND TEXTILE FLÄCHENGEBILDE
FIBRES ET TISSUS THERMOPLASTIQUES

(30) Priority: 03.12.1998 US 110803 P
(43) Date of publication of application: 10.10.2001
(73) Proprietor: DOW GLOBAL TECHNOLOGIES INC., Midland, Michigan 48674 (US)
(72) Inventor: WHITE, Jerry, E., Lake Jackson, TX 77566 (US); BECKERDITE, Michael, N., Lake Jackson, TX 77566 (US); MANG, Michael, N., Eden Prairie, MN (US); SUBRAMANIAN, Ramki, Houston, TX 77054 (US); MAUGANS, Rex, A., Lake Jackson, TX 77566 (US); BLANKENSHIP, Larry, T., Lake Jackson, TX 77566 (US); WINKLER, Marie, S., Lake Jackson, TX 77566 (US); RIPPLINGER, Eric, B., Lake Jackson, TX 77566 (US); THYNE, Thomas, C., Lake Jackson, TX 77566 (US)
(74) Representative: Casalonga, Axel
(86) International application number: PCT/US1999/028462
(87) International publication number: WO 2000/032854

(56) References cited:
- EP-A- 0 780 438
- WO-A-98/51728
- US-A- 4 337 330
- PATENT ABSTRACTS OF JAPAN vol. 1998, no. 03, 27 February 1998 (1998-02-27) & JP 09 302522 A (TORAY IND INC), 25 November 1997 (1997-11-25)
- PATENT ABSTRACTS OF JAPAN vol. 005, no. 184 (C-080), 21 November 1981 (1981-11-21) & JP 56 107017 A (NIPPON ESTER CO LTD), 25 August 1981 (1981-08-25)
- PATENT ABSTRACTS OF JAPAN vol. 005, no. 184 (C-080), 21 November 1981 (1981-11-21) & JP 56 107016 A (NIPPON ESTER CO LTD), 25 August 1981 (1981-08-25)
- PATENT ABSTRACTS OF JAPAN vol. 012, no. 358 (C-531), 26 September 1988 (1988-09-26) & JP 63 112725 A (NIPPON ESTER CO LTD), 17 May 1988 (1988-05-17)

## Description

The present invention relates to thermoplastic fibers and fabrics.

It is known to prepare fibers, yarns and fabrics from polystyrene, vinyl polymers, nylons, polyesters, polyolefins, or fluorocarbons. See, for example. U.S. Patents 4.181.762: 4,945,150; 4,909,975 and 5,071,917.

However, it still remains desirable to provide fibers prepared from polymers which have not been used as starting materials for the preparation of fibers, yarns and fabrics. These fibers have exceptional properties with respect to bonding, hydrophilicity and chemical resistance which is a special feature of epoxy-based polymers.

In a first aspect, the present invention is a fiber comprising at least one thermoplastic hydroxy-functionalized polyether and, optionally, a thermoplastic polymer which is not a hydroxy-functionalized polyether.

In a second aspect, the present invention is a bicomponent fiber having (1 a first component comprising a thermoplastic hydroxy-functionalized polyether or a blend of hydroxy-functionalized polyether and (2) a second component comprising a thermoplastic polymer which is not a hydroxy-functionalized polyether.

In a third aspect, the present invention is a method of forming a non-woven fabric by forming a web of at least one fibrous component and heating the web to cause bonding of fibrous components of the web, characterized in that at least one fibrous component comprises a thermoplastic hydroxy-functionalized polyether.

The fiber of the present invention can be a single component or a bicomponent fiber.

The single component fiber comprises at least one thermoplastic hydroxy-functionalized polyether and, optionally, a thermoplastic polymer which is not a hydroxy-functionalized polyether.

In general, the thermoplastic hydroxy-functionalized polyethers are prepared by the reaction of a dinucleophilic monomer with a diglycidyl ether, a diglycidyl ester or epihalohydrin.

Preferably, the thermoplastic hydroxy-functionalized polyether is selected from :
(1) polyetheramines having repeating units represented by the formula:
(2) hydroxy-functionalized polyethers having repeating units represented by the formula: or
(3) hydroxy-functionalized poly(ether sulfonamides) having repeating units represented by the formula: or R³ is hydrogen or alkyl; R⁷ and R⁹ are independently alkyl, substituted alkyl, aryl, substituted aryl; R⁸ is a divalent organic moiety which is primarily hydrocarbon; A is an amine moiety or a combination of different amine moieties; B is a divalent organic moiety which is primarily hydrocarbon; and m is an integer from 5 to 1000.

In the preferred embodiment of the present invention, A is 2-hydroxyethylimino-, 2-hydroxypropyl-imino-, piperazenyl, N,N'-bis(2-hydroxyethyl)-1,2-ethylenediimino; and B and R' are independently 1,3-phenylene, 1,4-phenylene; sulfonyldiphenylene, oxydiphenylene, thiodiphenylene or isopropylidene-diphenylene; R⁵ is hydrogen; R⁷ and R⁹ are independently methyl, ethyl, propyl, butyl, 2-hydroxyethyl or phenyl; and B and R⁸ are independently 1,3-phenylene, 1,4-phenylene, sulfonyldiphenylene, oxydiphenylene, thiodiphenylene or isopropylidenediphenylene.

The polyetheramines represented by Formula I also referred to as poly(hydroxy amino ethers), are prepared by contacting one or more of the diglycidyl ethers of a dihydric phenol with an amine having two amine hydrogens under conditions sufficient to cause the amine moieties to react with epoxy moieties to form a polymer backbone having amine linkages, ether linkages and pendant hydroxyl moieties. These polyetheramines are described in U.S. Patent 5.275.853. The polyetheramines can also be prepared by contacting a diglycidyl ether or an epihalohydrin with a difunctional amine

The hydroxy-functionalized polyethers represented by Formula II are prepared, for example, by contacting a diglycidyl ether or a combination of diglycidyl ethers with a dihydric phenol or combination of dihydric phenols using the process described in U.S. Patent 5,164,472. Alternatively, the poly(hydroxy ethers) are obtained by allowing a dihydric phenol or a combination of dihydric phenols to react with an epihalohydrin by the process described by Reinking, Barnabeo, and Hale in the *Journal of Applied Polymer Science, Volume 7, page 2135 (1963).*

The hydroxy-functionalized poly(ether sulfonamides) represented by Formulae IIIa and IIIb are prepared, for example, by polymerizing an N,N'-dialkyl or N,N'-diaryldisulfonamide with a diglycidyl ether as described in U.S. Patent 5,149,768.

The hydroxy-functionalized polyethers commercially available from Phenoxy Associates, Inc. are also suitable for use in the present invention. These hydroxy-functionalized polyethers are the condensation reaction products of a dihydric polynuclear phenol, such as bisphenol A, and an epihalohydrin and have the repeating units represented by Formula II wherein B is an isopropylidene diphenylene moiety. These hydroxy-phenoxyether polymers and the process for preparing them are described in U.S. Patents 3,305,528. Other hydroxy functional polyethers that are suitable for use in the present invention are poly(alkylene oxides), which are typically produced through the polymerization of ethylene oxide, propylene oxide or butylene oxide. Specific examples include, but are not limited to, poly(ethylene oxide), poly(propylene oxide), poly(butylene oxide), or copolymers containing varying amounts of different poly(alkylene oxides). These polymers also may be particularly suitable for blending with polymers of any of Formulas I through III. Advantages of blends of poly(alkylene oxides) and polymers of Formulas I through III include the ability to manipulate the glass transition temperature of the blends or to modify hydrophilicity.

The polymers which are not hydroxy-functionalized polyethers which can be employed in the practice of the present invention for preparing the fibers include polyolefins, polyesters, polyamides, polysaccharides, modified polysaccharides or naturally-occurring fibers or particulate fillers; thermoplastic polyurethanes, thermoplastic elastomers and glycol-modified copolyester (PETG). Other polymers of the polyester or polyamide type can also be employed in the practice of the present invention for preparing the fiber. Such polymers include poly(hexamethylene adipamide), polycaprolactone, poly(hexamethylene sebacamide), poly(ethylene 2,6-naphthalate) and poly(ethylene 1.5-naphthalate), poly(tetramethylene 1,2-dioxybenzoate) and copolymers of ethylene terephthalate and ethylene isophthalate.

The polyesters and methods for their preparation are well known in the art and reference is made thereto for the purposes of this invention. For purposes of art illustration and not limitation, reference is particularly made to pages 1-62 of Volume 12 of the *Encyclopedia of Polymer Science and Engineering,* 1988 revision, John Wiley & Sons.

The polymers which are not hydroxy-functionalized polyethers can be blended with the hydroxy-functionalized polyether at levels of less than 50 weight percent and, preferably less than 30 weight percent, based on the weight of the fiber. These other polymers can be blended into the hydroxy-functionalized polyether in order to reduce composition cost, to modify physical properties, barrier or permeability properties, or adhesion characteristics. In the case of bicomponent fibers, the separate non-hydroxy-functional-containing component may be used at levels of up to 99 percent, preferably less than 95 percent, based on the weight of the fiber.

The polyamides which can be employed in the practice of the present invention for preparing the fibers include the various grades of nylon, such as nylon 6, nylon 6,6 and nylon 12.

By the term "polyolefin" is meant a polymer or copolymer derived from simple olefin monomers such as ethylene, propylene, butylene, or isoprene, and one or more monomers copolymerizable therewith. Such polymers (including raw materials, their proportions, polymerization temperatures, catalysts and other conditions) are well-known in the art and reference is made thereto for the purpose of this invention. Additional comonomers which can be polymerized with ethylene include olefin monomers having from 3 to 12 carbon atoms, ethylenically unsaturated carboxylic acids (both mono-and difunctional) and derivatives of such acids such as esters (for example, alkyl acrylates) and.anhydrides; monovinylidene aromatics and monovinylidene aromatics substituted with a moiety other than halogen such as styrene and methylstyrene; and carbon monoxide. Exemplary monomers which can be polymerized with ethylene include 1-octene, acrylic acid, methacrylic acid, vinyl acetate and maleic anhydride.

The polyolefins which can be employed in the practice of the present invention for preparing the fibers include polypropylene, polyethylene, and copolymers and blends thereof, as well as ethylene-propylene-diene terpolymers. Preferred polyolefins are polypropylene, such as Pro-fax™ PF635 (Trademark of Montell North American Inc.) and INSPIRE™ (Trademark of The Dow Chemical Company), linear high density polyethylene (HDPE), heterogeneously-branched linear low density polyethylene (LLDPE) such as DOWLEX™ polyethylene resin (Trademark of The Dow Chemical Company), heterogeneousiy-branched ultra low linear density polyethylene (ULDPE) such as ATTANE™ ULDPE (Trademark of The Dow Chemical Company): homogeneously-branched, linear ethylene/α-olefin copolymers such as Tafmer™ (Trademark of Mitsui Petrochemicals Company Limited) and Exact™ (Trademark of Exxon Chemical Company); homogeneously branched, substantially linear ethylene/α-olefin polymers such as AFFINITY™ (Trademark of The Dow Chemical Company) and ENGAGE® (Trademark of DuPont Dow Elastomers L.L. C) polyolefin elastomers, which can be prepared as disclosed in U.S. Patents 5,272,236 and 5,278,272; and high pressure, free radical polymerized ethylene polymers and copolymers such as low density polyethylene (LDPE), ethylene-acrylic acid (EAA) copolymers such as PRIMACOR™ (Trademark of The Dow Chemical Company), and ethylene-vinyl acetate (EVA) copolymers such as Escorene™ polymers (Trademark of Exxon Chemical Company), and Elvax™ (Trademark of E.I. du Pont de Nemours & Co.). The more preferred polyolefins are the homogeneously-branched linear and substantially linear ethylene copolymers with a density (measured in accordance with ASTM D-792) of 0.85 to 0.99 g/cm³, a weight average molecular weight to number average molecular weight ratio (Mw/Mn) from 1.5 to 3.0, a measured melt index (measured in accordance with ASTM D-1238 (190/2.16)) of 0.01 to 100 g/10 minutes, and an 110/12 of 6 to 20 (measured in accordance with ASTM D-1238 (190/10)).

In general, high density polyethylene (HDPE) has a density of at least about 0.94 grams per cubic centimeter (g/cc) (ASTM Test Method D-1505). HDPE is commonly produced using techniques similar to the preparation of linear low density polyethylenes. Such techniques are described in U.S. Patents 2,825,721; 2,993,876; 3,250,825 and 4,204,050. The preferred HDPE employed in the practice of the present invention has a density of from 0.94 to 0.99 g/cc and a melt index of from 0.01 to 35 grams per 10 minutes as determined by ASTM Test Method D-1238.

The polysaccharides which can be employed in the practice of the present invention are the different starches, celluloses, hemicelluloses, xylanes, gums, pectins and pullulans. Polysaccharides are known and are described, for example, in *Encyclopedia of Polymer Science and Technology, 2nd edition, 1987* The preferred polysaccharides are starch and cellulose.

The modified polysaccharides which can be employed in the practice of the present invention are the esters and ethers of polysaccharides, such as, for example, cellulose ethers and cellulose esters, or starch esters and starch ethers. Modified polysaccharides are known and are described, for example, in *Encyclopedia of Polymer Science and Technology, 2*^{*nd*} *edition, 1987.*

The term "starch" as used herein, refers to carbohydrates of natural vegetable origin, composed mainly of amylose and/or amylopectin, and includes unmodified starches, starches which have been dewatered but not dried, physically modified starches, such as thermoplastic, gelatinized or cooked starches, starches with a modified acid value (pH) where acid has been added to lower the acid value of a starch to a range of from 3 to 6, gelatinized starches, ungelatinized starches, cross-linked starches and disrupted starches (starches which are not in particulate form). The starches can be in granular, particulate or powder form. They can be extracted from various plants, such as, for example, potatoes, rice, tapioca, corn, pea, and cereals such as rye, oats, and wheat.

Celluloses are known and are described, for example, in *Encyclopedia of Polymer Science and Technology, 2nd edition, 1987.* Celluloses are natural carbohydrate high polymers (polysaccharides) consisting of anhydroglucose units joined by an oxygen linkage to form long molecular chains that are essentially linear. Cellulose can be hydrolyzed to form glucose. The degree of polymerization ranges from 1000 for wood pulp to 3500 for cotton fiber, giving a molecular weight of from 160,000 to 560,000. Cellulose can be extracted from vegetable tissues (wood, grass, and cotton). Celluloses can be used in the form of fibers.

The naturally-occurring fibers or particulate fillers which can be employed in the practice of the present invention are, for example, wood flour, wood pulp, wood fibers, cotton, flax, hemp, or ramie fibers, rice or wheat straw, chitin, chitosan, cellulose materials derived from agricultural products, nut shell flour, corn cob flour, and mixtures thereof.

In general, the fibers of the present invention can be formed by well known processes such as melt spinning, wet spinning, or conjugate spinning. The fibers of the present invention may be extruded into any size, or length desired. They may also be extruded into any shape desired, such as, for example, cylindrical, cross-shaped, trilobal or ribbon-like cross-section.

The bicomponent fibers of the present invention can have the following fiber cross-section structures:
(1) Side-by-side
(2) Sheath-core
(3) Islands-in-the sea and
(4) Citrus (Segmented pie)

### (1) Side-by-side

A method for producing side-by-side bicomponent fibers is described in U.S. Patent 5,093,061. The method comprises (1) feeding two polymer streams through orifices separately and converging at substantially the same speed to merge side-by-side as a combined stream below the face of the spinneret; or (2) feeding two polymer streams separately through orifices, which converge at the surface of the spinneret, at substantially the same speed to merge side-by-side as a combined stream at the surface of the spinneret. In both cases, the velocity of each polymer stream at the point of merge is determined by its metering pump speed and the size of the orifice. The fiber cross-section has a straight interface between two components.

Side-by-side fibers are generally used to produce self-crimping fibers. All commercially available self-crimping fibers are produced by using a system based on the different shrinkage characteristics of each component.

### (2) Sheath-core

Sheath-core bicomponent fibers are those fibers where one of the components (core) is fully surrounded by a second component (sheath). Adhesion is not always essential for fiber integrity.

The most common way to produce sheath-core fibers is a technique in which two polymer liquids (melts) are separately led to a position very close to the spinneret orifices and then extruded in sheath-core form. In the case of concentric fibers, the orifice supplying the "core" polymer is in the center of the spinning orifice outlet and flow conditions of core polymer fluid are strictly controlled to maintain the concentricity of both components when spinning. Modifications in spinneret orifices enable one to obtain different shapes of core or/and sheath within the fiber cross-section.

The sheath-core structure is employed when it is desirable for the surface to have the property of one of the polymers such as luster, dyeability or stability, while the core may contribute to strength, and reduced cost. The sheath-core fibers are used as crimping fibers and as bonding fibers in the non-woven industry.

The sheath-core bicomponent fiber can have a core comprising the hydroxy-functionalized polyether or polyester and a sheath comprising a polymer which is not a hydroxy-functionalized polyether or polyester. Alternatively, the hydroxy-functionalized polyether or polyester can be the sheath and the polymer that is not the hydroxy-functionalized polyether or polyester the core of the bicomponent fiber. The sheath-core may be circular in cross-section or may have some other geometry, such as trilobal. A variant such as "tipped trilobal" can also be constructed wherein the sheath component is no longer continuous about the core but exists only at the tips of the lobes formed by the core. Other configurations which may be utilized are illustrated in *International Fiber Journal, Volume 13, No,* 3, *June* 1998 in the articles beginning on pages 20, 26, and 49.

Methods for producing sheath - core bicomponent fibers are described in U.S. Patents 3,315,021 and 3,316,336.

### (3) Islands-in the-sea

Islands-in-the sea fibers are also called matrix-filament fibers which include heterogeneous bicomponent fibers. A method for producing islands-in-the sea fibers is described in U.S. Patent 4,445,833. The method comprises injecting streams of core polymer into sheath polymer streams through small tubes with one tube for each core stream. The combined sheath-core streams converge inside the spinneret hole and form one island-in-the sea conjugate stream.

Mixing the different polymer streams with a static mixer in the spinning process also makes island-in-the-sea bicomponent fibers. The static mixer divides and redivides the polymer stream to form a matrix stream with multiple cores. This method for producing island-in-the-sea fibers is described in U.S. Patent 4,414,276.

The hydroxy-functionalized polyether or polyester can be the sea polymer and the polymer which is not a hydroxy-functionalized polyether or polyester can be the island polymer. The hydroxy-functionalized polyether or polyester can also be the island polymer and the polymer which is not a hydroxy-functionalized polyether or polyester, the sea polymer.

The islands-in-the-sea structure is employed when it is desirable to increase the modulus of the fiber, reduce moisture regain, reduce dyeability, improve the texturing capability or give the fiber a unique lustrous appearance.

### (4) Citrus type (Segmented pie)

The citrus type bicomponent or segmented pie bicomponent fibers can be made by polymer distribution and/or spinneret modifications of the pack assemblies employed in the methods described above for producing the side-by-side, sheath-core or islands-in-the-sea fibers. For example, by introducing a first polymer stream and a second polymer stream alternately through eight radial channels toward the spinneret hole instead of two channels, the resultant fiber is an eight-segment citrus type fiber. If the spinneret orifice has the configuration of three or four slots on a circle (a common orifice configuration to produce hollow fibers), the fiber is a hollow citrus type fiber with eight segments. The hollow citrus type fiber can also be made by the use of special spinneret orifice configurations with a sheath-core spin pack as described in U.S. Patents 4,246,219 and 4,357,290.

The fibers of the present invention can be blended with other synthetic or natural fibers, such as carbon fibers, cotton, wool, polyester, polyolefin, nylon, rayon, glass fibers, fibers of silica, silica alumina, potassium titanate, silicone carbide, silicone nitride, boron nitride, boron, acrylic fibers, tetrafluoroethylene fibers, polyamide fibers, vinyl fibers, protein fibers, ceramic fibers, such as aluminum silicate, and oxide fibers, such as boron oxide.

Additives such as pigments, stabilizers, impact modifiers, plasticizers, carbon black, conductive metal particles, abrasives and lubricating polymers may be incorporated into the fibers. The method of incorporating the additives is not critical. The additives can conveniently be added to the hydroxy-functionalized polyether or polyester prior to preparing the fibers. If the hydroxy-functionalized polyether or polyester is prepared in solid form, the additives can be added to the melt prior to preparing the fibers.

The fibers of the present invention can be crosslinked by chemical treatment, heating or irradiation with ultraviolet light. For example, the fibers can be chemically treated with crosslinking agents such as diisocyanates, glycidylmethacrylate, bisepoxides and anhydrides.

The fibers of the present invention are suitable for use in filtration media, binder fibers for glass or carbon fibers, binder fibers in non-woven fabrics made of thermoplastic polymers which are not hydroxy-functionalized polyethers or polyesters or binder fibers in non-woven fabrics made of cellulosic-based materials. These fibers are also useful in the manufacture of medical apparels. They are also useful in making woven and non-woven fabrics which can be used in making apparels, water-absorbent cloths, antistatic wipes, or water-absorbent mats.

Woven fabrics are formed from the fibers of the present invention by techniques commonly used in the woven textiles industry, such as weaving or knitting.

Non-woven fabrics are based on a fibrous web. The fibers of the present invention can be formed into webs using the following known technologies:
(1) Dry-formed, carded or air-laid and bonded - The webs are formed from staple fibers by carding or air-laying, bonded overall or in a pattern with latex or other water-borne adhesives. In carding, clumps of staple fibers are separated mechanically into individual fibers and formed into a coherent web. In air-laying, fibers are introduced into an airstream and are captured on a screen from the air stream.
(2) Thermal-bonded - Dry-formed webs of staple fibers are bonded with fusible fibers or composed entirely of fusible fibers.
(3) Air-laid - Wood pulp fibers, with or without added staple fibers, are bonded with latex or similar adhesives.
(4) Wet-formed - Short fibers are formed into a web by processes derived from paper-making technology, followed by bonding with latex or thermal binders.
(5) Spun-bonded - Webs composed of long filaments with normal textile diameter are formed directly from bulk polymer and are usually bonded thermally.
(6) Melt-blown - Webs of long, extremely fine diameter fibers are formed directly from bulk polymer and are usually bonded by hot embossing processes.
(7) Spun-laced - Dry-formed webs are mechanically entangled by multiple fine, high pressure water jets, in most cases, without adhesive binder.
(8) Needle-punched - Fibers are mechanically entangled by multiple reciprocating banks of barbed needles.
(9) Laminated - Different layers are combined in composite or reinforced fabric by an adhesive, thermal fusion or entanglement.
(10) Stitch-bonded - Staple fiber webs are reinforced or mechanically entrapped by yarns stitched or knitted through the webs.

Non-woven fabrics and processes for preparing them are described in the *Encyclopedia of Polymer Science And Engineering,* Second Edition, Volume 10, pages 204-251.

The following working examples are given to illustrate the invention and should not be construed as limiting its scope. Unless otherwise indicated, all parts and percentages are by volume.

### Example 1

A 3/8-inch (0.95 cm) single-screw extruder fitted with an 8-hole spinneret was used to spin monofilaments based on 100 percent thermoplastic hydroxy-functional polyether. The melt temperature was 200°C. The fibers were rolled onto bobbins without further stretching.

### Example 2

Bicomponent fibers containing polypropylene as the core and a thermoplastic hydroxy-functionalized polyether as the sheath were spun. Two single-screw extruders, one feeding the polypropylene and another feeding the thermoplastic hydroxy-functionalized polyether were used. The extruders fed the molten polymers (melt temperature was 200°C) to a 288-holed spinneret from which the bicomponent fibers were spun. Fibers with polypropylene:thermoplastic hydroxy-functionalized polyether ratios of 90:10, 80:20, 70:30, 40:60 and 50:50 were spun. The fibers were also stretched after exiting the spinneret by using extender rolls and then taken up on bobbins.

### Example 3

A polyetheramine poly(hydroxy amino ether) (derived from the reaction of the diglycidyl ether of bisphenol A and ethanolamine) and a polypropylene were spun into bicomponent fibers. The poly(hydroxy amino ether) had an MFI (Melt Flow Index) of 8 at 230°C using a 2.16 kg weight. The polypropylene source was a 35 MFI Pro-fax ™ PF635 polypropylene from Montell. This sheath/core bicomponent fiber was produced under the conditions listed in Table I.

### Example 4

A 30/70 weight/weight (w/w) poly(hydroxy amino ether) (derived from the reaction of the diglycidyl ether of bisphenol A and ethanolamine) sheath/polypropylene core bicomponent fiber was treated on a Tech Tex texturizing unit to impart a crimp . This equipment uses the stuffer box method of texturizing. The texturized yam was cut into staple fiber of 2-inch (5 cm) length on an Ace Strip Cutter, Model C-75. After the crimping and staple cutting operations the fiber was opened a 12-inch (30.5 cm) wide microdenier metallic card in lots of 30 grams. The open fiber was then used to produce a batt on a sample card line. This carded batt was needled on a James Hunter Fiberlocker Needle machine to give a resultant needle-punched fabric.

### Example 5

Cotton fibers (4 kg, 1.5 to 5 cm in length) and 7-denier bicomponent fibers (30/70 (w/w) poly(hydroxyaminoether)/polypropylene), (0.45 kg, 2.5 cm in length) were manually mixed and then opened up. The blend was carded and converted into a non-woven web, which was thermally bonded with calender rolls at 170°C.

### Example 6

Cotton linters (150 g) and 7-denier bicomponent fibers (30/70 (w/w) polyetheramine/polypropylene) were added to 300 L of water in a cylindrical tank and the contents were agitated for 5 minutes. The polyetheramine was derived from the reaction of the diglycidyl ether of bisphenol A and ethanolamine. The ratio of bicomponent fibers to cotton linters was 5 percent on a weight basis. The slurry was then pumped to a moving belt made of polyester mesh and the webs formed were collected. The wet webs were dried by passing them through a 165°C oven with approximately one minute of dwell time. The dried webs were then bonded with heated calender rolls at temperatures from 100°C to 180°C. The basis weight of the webs after bonding was about 90 gsm.

### Example 7

A bicomponent, sheath/core spunbond fabric was produced under the conditions shown in Table II. The polyetheramine (derived from the reaction of the diglycidyl ether of bisphenol A and ethanolamine) sheath had a MFI of 15. The polypropylene core was composed of a 35 MFI Pro-fax ™ PF635. The sheath/core ratio was 20/80 (w/w). The system was run at slot air pressures of 20, 25 and 30 psi and the spunbond material was collected on perforated belt/vacuum collection system. Collection speeds ranged from 50 to 75 meters per minute. Calender rolls were set to 60°C and appeared to provide adequate bonding for dry web stock.

### Examples 8 Through 15 - PHAE Blends for Hydrophilic Fiber/Fabric Applications

The poly(hydroxy amino ether) ("PHAE") used in the following Examples 8 through 15 was produced by The Dow Chemical Company from the polymerization of a diglycidyl ether of Bisphenol A and ethanol amine. The PHAE had the following properties: number average molecular weight (Mn) = 14,000; weight average molecular weight (Mw) = 35,000; melt index =15 (measured at 190°C with a 2.16 kg weight); glass transition temperature (Tg) = 78°C. In these Examples 8 through 15, PEG refers to poly(ethylene glycol) and PEO refers to poly(ethylene oxide). PEG and PEO have the same polyoxyethylene repeating unit shown below:

(-CH₂CH₂O-)ₙ

Designation of polymers with the above structure as PEG or PEO was based on the product name given in an Aldrich catalogue, that is, PEG is used if the number average molecular weight (Mn) of the polyoxyethylene is 10,000 or less, and PEO if the viscosity average molecular weight (Mv) is 100,000 or above. In the following examples, the number immediately after PEG or PEO indicates the calculated average molecular weight (Mn or Mv) from the Aldrich catalog.

EPE refers to a block copolymer with the general structure shown below:

H(-OCH₂CH₂-)ₓ[-OCH(CH₃)CH₂-]_{y}(-OCH₂CH₂-)_{z}OH

The EPE block copolymers contain a hydrophobic block of poly(propylene oxide), having a molecular weight ranging from a minimum of 900 to a maximum of 4000, with two hydrophilic polyoxyethylene blocks such that the combined weight of the polyoxyethylene blocks constitutes from 10 to 90 weight percent of the total molecule. The EPE block copolymers are nonionic surfactants [see L. G. Lundsted and I. R. Schmolka, "The Synthesis and Properties of Block Copolymer Polyol Surfactants" in *Block and Graft Copolymerization, volume* 2 (edited by R. J. Ceresa), John Wiley and Sons, New York, chapter 1, pp. 1-103]. The EPE block copolymers are marketed under the Trademark PLURONIC® polyols (BASF Wyandotte Corporation) and are also sold by The Dow Chemical Co. (for example, Polyglycol EP-1730 and EP-1660).

The nomenclature used herein for specific EPE block copolymers gives the weight percent ethylene glycol and the average calculated molecular weight (Mn), as given in the Aldrich catalog. For example, EPE-30 (Mn 5800) refers to an EPE block copolymer containing 30 weight percent ethylene glycol and having a calculated number average molecular weight of 5800.

The following test methods were used for Examples 8 through 15

Glass transition temperature (Tg) was determined using a TA Instruments DSC 2010 Differential Scanning Calorimeter. Samples (5 to 10 mg) were prepared in hermetically sealed pans. Two scans were made for each sample. The first scan was made from ambient to 200°C at 10°C per minute. The sample was then cooled to ambient temperature or below using dry ice, whereupon the second scan was made at 10°/minute to 200°C. The Tg was determined from the second scan inflection point.

pH7 Buffer Contact Angle was determined for compression molded films using a Krüss G40 Contact Angle Measuring System (Goniometer) equipped with a Eurometrix fiber optic light source, a Kernco model G-1 microscope, stage, light source, and camera mount, and a Kruss Panasonic CCTV camera and WV-5410 monitor. A small drop of the pH7 buffer was applied to the film and the angle formed at the film/drop/air interface was measured using the system software (G40 V1.32-US). In the examples that follow the terms "water contact angle" and "pH7 buffer contact angle" are synonymous.

Laboratory-scale fiber spinning of PHAE blends. The apparatus for spinning fiber consisted of a Rheometrix capillary melt rheometer equipped with a 1000 µm die, a Rheotens attachment, and a 12 inch (30.5 cm) circumference variable speed roll onto which the fiber was spun.

### Example 8 - PHAE Blend With 10 Weight Percent PEG 10.000

PHAE (243.0 g) and PEG 10,000 (27.1 g, Aldrich Chemical Co., Tm 63°C) were melt blended for 20 minutes in a large capacity Haake Torque rheometer (with roller mixing blades) at 170°C isothermal metal temperature and 100 rpm mixing rate. The resulting blend had a Tg of 53°C with no crystalline melting point. A compression molded film of the blend was transparent and had a water contact angle of 67. Fiber was melt spun at 190°C with a rheometer plunger speed of 0.3 inch/minute and a take-up roll speed of 1780 rpm (543 m/minute). Additional blends with 5 and 25 weight percent PEG 10,000 were also prepared and the results are included in Table III.

### Example 9 - PHAE Blend With 5 Weight Percent PEO 100.000

PHAE (57.1 g) and PEO 100,000 (3.1 g, Aldrich Chemical Co., Tm 65°C) were melt blended in a Haake Torque rheometer for 15 minutes at 180°C isothermal metal temperature and 100 rpm mixing rate. The resulting blend had a Tg of 66°C with no crystalline melting point. A compression molded film of the blend was transparent and had a water contact angle of 68. Fiber was melt spun at 190°C with a plunger speed of 0.3 inch/minute (8mm/minute) and a take-up speed of 1780 rpm (543 m/minute). The denier of the fiber was 9 g (equals the weight of 9000 m of continuous fiber). Additional blends with 10 percent and 25 percent PEO 100,000 were prepared and the results are included in Table III.

### Example 10 - PHAE blend with 5 Weight Percent PEO 4.000.000

PHAE (57.0 g) and PEO 4,000,000 (3.0 g, Aldrich Chemical Co., Tm 65°C) were melt blended in a Haake torque rheometer for 20 minutes at 180°C isothermal metal temperature and 100 rpm mixing rate. The resulting blend had a Tg of 67°C with no crystalline melting point. A compression molded film of the blend was transparent and had a water contact angle of 65. Fiber was melt spun at 190°C with a plunger speed of 0.3 inch/minute (8 mm/minute) and a take-up speed of 1780 rpm (543 m/minute). The denier of the fiber was 10 g.

### Example 11 - PHAE Blend With 10 Weight Percent PEO 4.000.000

PHAE (243.0 g) and PEO 4,000,000 (27.0 g, Aldrich Chemical Co., Tm 65°C) were melt blended in a Haake torque rheometer for 25 minutes at 180°C isothermal metal temperature and 100 rpm mixing speed. The resulting blend had a Tg of 55°C with no crystalline melting point. A compression molded film of the blend was transparent and had a water contact angle of 72. Fiber was melt spun at 190°C with a plunger speed of 0.3 inch/minute (8 mm/minute) and a take-up speed of 1780 rpm (543 m/minute).

### Example 12 - PHAE Blend With 15 Weight Percent PEO 4,000,000

PHAE (51.0 g) and PEO 4,000,000 (9.0 g, Aldrich Chemical Co., Tm 65°C) were melt blended in a Haake torque rheometer for 20 minutes at 180°C isothermal metal temperature and 100 rpm mixing rate. The resulting blend had a Tg of 44°C with no crystalline melting point. A compression molded film of the blend was transparent and had a water contact angle of 42. Fiber was melt spun at 190°C with a plunger speed of 0.3 inch/minute (8 mm/minute) and a take-up speed of 1100 rpm (335 m/minute). Additional blends with 20 and 25% PEO 4,000,000 were prepared and the results are included in Table III.

### Example 13 - PHAE Blend With 3.7 Weight Percent EPE-30 (Mn 5800)

PHAE (73.4 g) and EPE-30 (2.8 g, Aldrich Chemical Company, Tm 39°C) were melt blended in a Haake torque rheometer for 20 minutes at 180°C isothermal metal temperature and 100 rpm mixing rate. The resulting blend had a Tg of 69°C with no crystalline melting point. A compression molded film of the blend had a pearlescent, semi-transparent appearance and had a water contact angle of 24. Fiber was melt spun at 200°C with a plunger speed of 0.3 inch/minute and a take-up speed of 1780 rpm (543 m/minute). The denier of the fiber produced was 8g. A small hand sample of fabric was made from the fiber as follows: A portion of the fiber (1.4 g) was cut into 2 inch staple and carded to make a web. The web was folded in half and then run through a Beloit Wheeler Model 700 Lab Calendar Roll. The calender rolls were set at 210°F and 1000 psi which gave a well bonded fabric. A sample of pure PHAE fiber (1.4 g) was made into fabric using a similar procedure. The ability of the fabrics to wick water was then tested by immersing one end of a small strip (19 by 81 mm) of each fabric into deionized water and measuring the time required for the water to advance up the fabric strip to a line drawn 25 mm from the surface of the water. The PHAE blend with EPE-30 (Mn 5800) wicked water to the line in 2.5 minutes whereas the pure PHAE fabric showed no wicking of water at all. The fabrics were redried and the wicking test was repeated 3 times. The same results were observed each time - the fabric made with the EPE-30 blend wicked water and the pure PHAE fabric did not.

### Example 14 - PHAE blend with 5 Weight Percent EPE-80 (Mn 8400)

PHAE (57.0 g) and EPE-80 (3.0 g, Aldrich Chemical Co., Tm 58°C) were melt blended in a Haake torque rheometer for 20 minutes at 180°C isothermal metal temperature and 100 rpm mixing rate. The resulting blend had a Tg of 64°C with no crystalline melting point. A compression molded film of the blend was transparent and had a water contact angle of 56. Fiber was melt spun at 200°C with a plunger speed of 0.3 inch/minute and a take-up speed of 850 rpm (259 m/minute). The denier of the fiber produced was 274g.

Blends of PHAE with other EPE block copolymers, including EPE-30 (Mn 4400); EPE-40 (Mn 2,900); and EPE-50 (Mn 1,900), were also prepared using procedures analogous to those described above. The results for these blends are listed in Table IV.

### Example 15 - PHAE blend with 5 Weight Percent Poly(propylene glycol) (Aldrich. Mn 3500)

PHAE (64.9 g) and poly(propylene glycol) (3.4 g) were melt blended in a Haake torque rheometer for 40 minutes at 150°C to 180°C isothermal metal temperature and 30 to 100 rpm mixing rate. The initial blend appeared to be two-phase and mixing was very poor. Temperature and mixing rate were adjusted until good mixing was obtained. The resulting blend had a Tg of 76°C. A compression molded film of the blend was opaque.

**Table III PHAE Blends with Polyoxyethylene (PEG or PEO)**

| PHAE blend composition (a) | Tg °C | Contact angle (pH7 buffer) (b) | Comment (c) |
|---|---|---|---|
| pure PHAE | 78 | 89 ± 5 | |
| 5% PEG 10,000 | 64 | 68 ±4 | miscible |
| 10% PEG 10,000 | 53 | 67 ±3 | " |
| 25% PEG 10,000 | 20 | 23 ±5 | " |
| 5% PEO 100,000 | 66 | 68 ± 6 | miscible |
| 10% PEO 100,000 | 54 | 64 ± 4 | " |
| 25% PEO 100,000 | 21 | 25 ± 8 | " |
| 5% PEO 4,000,000 | 67 | 65 ± 4 | miscible |
| 10% PEO 4,000,000 | 55 | 67 ±3 | **"** |
| 15% PEO 4,000,000 | 44 | 42 ± 6 | " |
| 20% PEO 4,000,000 | 37 | 18±4 | " |
| 25% PEO 4,000,000 | 21 | 17 ±3 | " |

| | | | |
|---|---|---|---|
| a) Weight percent of additive given with the balance being PHAE. | | | |
| b) Contact angle measurement for drops of pH 7 buffer solution applied to the surface of a compression molded film. Value reported is the average of results for 15 drops. | | | |
| c) Samples were classified as miscible if the Tg satisfied the Fox equation and if films of the blends were transparent. | | | |

**Table IV PHAE blends with EPE Block Copolymers**

| PHAE blend composition (a) | Tg, °C | Contact angle (pH7 buffer) (b) | Comment (c) |
|---|---|---|---|
| Pure PHAE | 78 | 89 ± 5 | Fiber made at high iine speed: denier = 7, Fabric sample does not wick water |
| 3.7% EPE-30 (Mn 5,800) | 69 | 24 ± 2 | Immiscible blend; Fiber made at high speed: diameter = 30µm; Fabric sample exhibits wicking of water |
| 2% EPE-30 (Mn 4,400) | 78 | 46 ± 5 | Immiscible blend |
| 4% EPE-30 (Mn 4,400) | 76 | 37 ± 2 | " |
| 2% EPE-40 (Mn 2,900) | 75 | 31 ± 4 | Immiscible blend |
| 4% EPE-40 (Mn 2,900) | 73 | 24 ± 3 | " |
| 2% EPE-50 (Mn 1,900) | 73 | 73 ± 3 | Miscible blend |
| 5% EPE-50 (Mn 1,900) | 65 | 34 ± 5 | " |
| 5% EPE-80 (Mn 8,400) | 64 | 56 ± 4 | Miscible blend; Fiber made at medium speed |
| 10% EPE-80 (Mn 8,400) | 55 | 56 ± 3 | " |

| | | | |
|---|---|---|---|
| a) Weight percent of additive given with the balance being PHAE. | | | |
| b) Contact angle measurement for drops of pH 7 buffer solution applied to the surface of a compression molded film. Value reported is the average of results for 15 drops. | | | |
| c) Samples were classified as miscible if the Tg satisfied the Fox equation and if films of the blends were transparent. | | | |

## Claims

1. A fiber comprising at least one thermoplastic hydroxy-functionalized polyether selected from:
(1) polyetheramines having repeating units represented by the formula:
(2) hydroxy-functionalized polyethers having reapeating units represented, by the formula: or
(3) hydroxy-functionalized poly(ether sulfonamides) having repeating units represented by the formula: or wherein
R⁵ is hydrogen or alkyl; and R⁹ are independently alkyl, substituted alkyl, aryl, substituted aryl; R⁸ is a divalent organic moiety Which is primarity hydrocarbon; A is art amine moiety or a combination of different amine moieties; B Is a divalent organic moiety which is primanly hydrocarbon; and m is an integer from 5 to 1000.

2. The fiber of Claim 1 wherein the thermoplastic hydroxy-functionalized polyether is prepared by the reaction of a dinucleophilic monomer with a diglyciclyl ether, a diglycidyl ester or epihalohydrin.

3. The fiber of Claim 1 having a cylindrical, cross-shaped, trilobal or ribbon-liks cross-section.

4. The fiber of Claim 1 formed by melt-spinning, dry-spinning or wet-spinning of a polymer solution.

5. The fiber of Claim 1 in the form of a filtration medium, a binder fiber for glass or carbon fibers, a binder fiber in non-woven fabrics made of a thermoplastic polymer which is not a hydroxy-functionalized polyether or a binder fiber in non-woven fabrics made of cellulosic-based materials, or a medical apparel.

6. A woven or non-woven fabric comprising the fiber of Claim 1 and, optonially, a synthetic or natural fiber.

7. The fabric of Claim 6 wherein the synthetic fiber is a polyester, a polyamide, rayon or a polyolefin and the, natural fiber Is cotton.

8. The fabric of Claim 6 in the form of an apparel, a water-absorbent cloth, a filter fabric, a battery separator, an antistatic wipe or a water-absorbent mat.

9. The fiber of Claim 1 comprising a blend or one of more hydroxy-functionalized polyether with a thermoplastic polymer which is not an hydroxy-functionalized polyether selected from a polyolefin, polyester, polyamide, polysaccharide, modified polysaccharide or naturally-occurring fiber or particulate filler, thermoplastic polyurethane, thermoplastic elastomer or glycoi-modified copolyester (PETG).

10. The fiber of Claim 1 which Is a bicomponent fiber having (1) a first component comprising a thermoplastic hydroxy-functionalized polyether or a blend of a hydroxy-functionalized polyether and (2) a second component comprising a polyolefin, polyester, polyamide, polysaccharide, modified polysaccharide or naturally-occurring fiber or particulate filler, thermoplastic polyurethane, thermoplastic elastomer or glycol-modified copolyester (PETG).

11. The bicomponent fiber of Claim 10 wherein the hydroxy-functionalized polyether is prepared by the reaction of a dinucleophilic monomer with a diglycidyl ether, a diglycidyl ester or eplhalohydrin.

12. The bicomponent fiber of Claim 10 or 11 which is a side-by-side bicomponent fiber, a sheath-core bicomponent fiber, a segmented-pie bicomponent fiber or an islands-in-the-sea bicomponent fiber.

13. The bicomponent fiber of Claim 12 comprising a core of the thermoplastic hydroxy-functionalized polyether and a sheath of a thermoplastic polymer which is not a hydroxy-functionalized polyether.

14. The bicomponent fiber of Claim 12 comprising a sheath of the thermoplastic hydroxy-functionalized polyether and a core of a thermoplastic polymer which is not a hydroxy-functionalized polyether or polyester.

15. The bicomponent fiber of Claim 11 having a cyndrical, cross-shaped, trilobal or ribbon-like cross-section.

16. The bicomponent fiber of Claim 11 in the form of a filtration medium, a binder fiber for glass or carbon fibers, a binder fiber in non-woven fabrics made of a thermoplastic polymer which is not a hydroxy-functionalized polyether or polyester or a binder fiber in non-woven fabrics made of cellulosic-based materials, or a medical apparel.

17. A woven or non-woven fabric comprising the fiber of Claim 11 and, optionally, a synthetic or natural fiber.

18. The fabric of Claim 17 wherein the synthetic fiber is a polyester, a polyamide, rayon or a polyolefin and the natural liber is cotton.

19. The fabric or Claim 17 in the form of an apparel, a water-absorbent cloth, a filter fabric, a battery separator, an antistatic wipe or a water-absorbent mat

20. The fiber of Claim 1 comprising a blend of:
(a) a poly(hydroxy amino ether) having repeating units represented by the formula: wherein A is a diamino moiety or a combination of different amine moieties; B is a divalent organic moiety which is predominantly hydrocarbylene; R is alkyl or hydrogen; and n is an integer from 5 to 1000 and
(b) at least one of a polyethylene glycol, poly(ethylene oxide), or EPE block copolymer.

21. The fiber of claim 20 wherein the poly(hydroxy amino ether) is the reaction product of a diglycidyl ether of bisphenol-A and ethanolamine.

22. A method of forming a non-woven fabric by forming a web of at least one fibrous component and heating the web to cause bonding of fibrous components of the web, **characterized in that** at least one fibrous component comprises a thermoplastic hydroxy-functionalized polyether according to claim 1.

23. The method of Claim 22 wherein at least one fibrous component comprises a poly(hydroxy amino ether) having repeating units represented by the formula: wherein A is a diamino moiety or a combination of different amine moieties; B is a divalent organic moiety which is predominantly hydrocarbylene; R is alkyl or hydrogen; and n is an integer greater than 10.

## Revendications

1. Fibre comprenant au moins un polyéther à fonction hydroxy thermoplastique choisi parmi :
(1) les polyétheramines ayant des unités répétitives représentées par la formule :
(2) les polyéthers à fonction hydroxy ayant des unités répétitives représentées par la formule : ou
(3) les poly(éther sulfonamides) à fonction hydroxy ayant des unités répétitives représentées par la formule :
dans lesquelles
R⁵ représente un atome d'hydrogène ou un groupe alkyle ; R⁷ et R⁹ représentent indépendamment un groupe alkyle, alkyle substitué, aryle, aryle substitué ; R⁸ représente un groupe organique divalent qui est principalement un hydrocarbure ; A représente un groupe amine ou une combinaison de différents groupes amine ; B représente un groupe organique divalent qui est principalement un hydrocarbure ; m représente un nombre entier de 5 à 1000.

2. Fibre conformément à la revendication 1 dans laquelle le polyéther à fonction hydroxy thermoplastique est préparé par la réaction d'un monomère dinucléophile avec un éther diglycidylique, un ester diglycidylique ou une épihalohydrine.

3. Fibre conformément à la revendication 1 ayant une section en coupe cylindrique, en forme de croix, trilobique ou de type ruban.

4. Fibre conformément à la revendication 1 formée par filage à chaud, filage à sec ou filage au mouillé d'une solution de polymères.

5. Fibre conformément à la revendication 1 sous la forme d'un milieu de filtration, d'une fibre liante pour les fibres de verre ou de carbone, d'une fibre liante dans les étoffes non tissées faites d'un polymère thermoplastique qui n'est pas un polyéther à fonction hydroxy ou d'une fibre liante dans les étoffes non tissées faites de matériaux à base de cellulose, ou d'un habillement médical.

6. Etoffe tissée ou non tissée comprenant la fibre conformément à la revendication 1 et optionnellement, une fibre synthétique ou naturelle.

7. Etoffe selon la revendication 6 dans laquelle la fibre synthétique est un polyester, un polyamide, la rayonne ou une polyoléfine et la fibre naturelle est le coton.

8. Etoffe selon la revendication 6 sous la forme d'un habillement, d'un tissu absorbant l'eau, d'une étoffe filtrante, d'un séparateur, d'un chiffon antistatique ou d'un mat absorbant l'eau.

9. Fibre selon la revendication 1 comprenant un mélange d'un ou plusieurs polyéthers à fonction hydroxy avec un polymère thermoplastique qui n'est pas un polyéther à fonction hydroxy choisi parmi une polyoléfine, un polyester, un polyamide, un polysaccharide, un polysaccharide modifié ou une fibre ou une charge particulaire naturelles, un polyuréthane thermoplastique, un élastomère thermoplastique ou un copolyester modifié par un glycol (PETG).

10. Fibre selon la revendication 1 qui est une fibre à deux composants ayant (1) un premier composant comprenant un polyéther à fonction hydroxy thermoplastique ou un mélange de polyéthers à fonction hydroxy et (2) un second composant comprenant une polyoléfine, un polyester, un polyamide, un polysaccharide, un polysaccharide modifié ou une fibre ou une charge particulaire naturelles, un polyuréthane thermoplastique, un élastomère thermoplastique ou un copolyester modifié par un glycol (PETG).

11. Fibre à deux composants selon la revendication 10 dans laquelle le polyéther à fonction hydroxy est préparé par la réaction d'un monomère dinucléophile avec un éther diglycilique, un ester diglycidylique ou une épihalohydrine.

12. Fibre à deux composants selon la revendication 10 ou 11 qui est une fibre à deux composants côte à côte, une fibre à deux composants gaine-coeur, une fibre à deux composants de type tarte segmentée ou une fibre à deux composants en îlots.

13. Fibre à deux composants selon la revendication 12 comprenant un coeur du polyéther à fonction hydroxy thermoplastique et une gaine d'un polymère thermoplastique qui n'est pas un polyéther à fonction hydroxy.

14. Fibre à deux composants selon la revendication 12 comprenant une gaine du polyéther à fonction hydroxy thermoplastique et un coeur d'un polymère thermoplastique qui n'est pas un polyéther ou un polyester à fonction hydroxy.

15. Fibre à deux composants selon la revendication 11 ayant une section en coupe cylindrique, en forme de croix, trilobique ou de type ruban.

16. Fibre à deux composants selon la revendication 11 sous la forme d'un milieu de filtration, d'une fibre liante pour les fibres de verre ou de carbone, d'une fibre liante dans les étoffes non tissées faites d'un polymère thermoplastique qui n'est pas un polyéther à fonction hydroxy ou d'une fibre liante dans les étoffes non tissées faites de matériaux à base de cellulose, ou d'un habillement médical.

17. Etoffe tissée ou non tissée comprenant la fibre selon la revendication 11 et, optionnellement, une fibre synthétique ou naturelle.

18. Etoffe selon la revendication 17 dans laquelle la fibre synthétique est un polyester, un polyamide, la rayonne ou une polyoléfine et la fibre naturelle est le coton.

19. Etoffe selon la revendication 17 sous la forme d'un habillement, d'un tissu absorbant l'eau, d'une étoffe filtrante, d'un séparateur, d'un chiffon antistatique ou d'un mat absorbant l'eau.

20. Fibre selon la revendication 1 comprenant un mélange de :
(a) un poly(hydroxy amino éther) ayant des unités répétitives représentées par la formule : dans laquelle A représente un groupe diamino ou une combinaison de différents groupes amine ; B représente un groupe organique divalent qui est principalement un groupe hydrocarbylène ; R représente un groupe alkyle ou un atome d'hydrogène ; et n représente un nombre entier de 5 à 1000 ; et
(b) au moins l'un d'un polyéthylène glycol, d'un poly(oxyde d'éthylène), ou d'un copolymère séquencé EPE.

21. Fibre selon la revendication 20 dans laquelle le poly(hydroxy amino éther) est le produit de réaction d'un éther diglycidylique de bisphénol-A et d'éthanolamine.

22. Procédé de formation d'une étoffe non tissée par formation d'une étoffe d'au moins un composant fibreux et chauffage de l'étoffe pour entraîner la liaison des composants fibreux de l'étoffe, **caractérisé en ce qu'**au moins un composant fibreux comprend un polyéther à fonction hydroxy thermoplastique selon la revendication 1.

23. Procédé selon la revendication 22 dans lequel au moins un composant fibreux comprend un poly(hydroxy amino éther) ayant des unités répétitives représentées par la formule : dans laquelle A représente un groupe diamino ou une combinaison de différents groupes amine ; B représente un groupe organique divalent qui est principalement un groupe hydrocarbylène ; R représente un groupe alkyle ou un atome d'hydrogène ; et n est un nombre entier supérieur à 10.

## Patentansprüche

1. Faser aus mindestens einem thermoplastischen hydroxyfunktionalisierten Polyether, der ausgewählt ist aus:
(1) Polyetheraminen mit Grundeinheiten, die repräsentiert werden durch die Formel:
(2) hydroxyfunktionalisierten Polyethern mit Grundeinheiten, die repräsentiert werden durch die Formel: oder
(3) hydroxyfunktionalisierten Poly(ethersulfonamiden) mit Grundeinheiten, die repräsentiert werden durch die Formel: oder
wobei R⁵ Wasserstoff oder Alkyl ist; R⁷ und R⁸ unabhängig voneinander Alkyl, substituiertes Alkyl, Aryl, substituiertes Aryl sind; R⁹ eine zweiwertige organische Komponente ist, die hauptsächlich Kohlenwasserstoff ist; A eine Aminkomponente oder eine Kombination von verschiedenen Aminkomponenten ist; B eine zweiwe r-tige organische Komponente ist, die hauptsächlich Kohlenwasserstoff ist; und m eine ganze Zahl von 5 bis 1000 ist.

2. Faser nach Anspruch 1, bei der der thermoplastische hydroxyfunktionalisierte Polyether hergestellt wird durch Umsetzen eines dinucleophilen Monomers mit einem Diglycidylether, einem Diglycidylester oder Epihalogenhydrin.

3. Faser nach Anspruch 1 , die einen zylindrischen, kreuzförmigen, trilobalen oder bändchenartigen Querschnitt hat.

4. Faser nach Anspruch 1, die durch Schmelzspinnen, Trockenspinnen oder Nassspinnen einer Polymerlösung gebildet wird.

5. Faser nach Anspruch 1 in Form eines Filtermediums, einer Bindefaser für Glas- oder Kohlenstofffasern, einer Bindefaser in Vliesstoffen aus einem therm o-plastischen Polymer, das kein hydroxyfunktionalisierter Polyether ist, oder einer Bindefaser in Vliesstoffen aus Materialien auf Cellulosebasis oder in Form eines medizinischen Kleidungsstücks.

6. Web- oder Vliesstoff, der die Faser nach Anspruch 1 und, fakultativ, eine Synthese- oder Naturfaser umfasst.

7. Stoff nach Anspruch 6, bei dem die Synthesefaser ein Polyester, ein Pol y-amid, Reyon oder ein Polyolefin ist und die Naturfaser Baumwolle ist.

8. Stoff nach Anspruch 6 in Form eines Kleidungsstücks, eines wasserabsorbierenden Tuchs, eines Filtergewebes, eines Batterietrennelements, eines antist a-tischen Lappens oder einer wasserabsorbierenden Matte.

9. Faser nach Anspruch 1 aus einer Mischung von ein oder mehr hydroxyfunktionalisierten Polyethern mit einem thermoplastischen Polymer, das kein hydroxyfunktionalisierter Polyether ist und ausgewählt ist aus einem Polyolefin, Polyester, Polyamid, Polysaccharid, modifiziertem Polysaccharid oder natürlich vorkommender Faser oder partikulärem Füllstoff, thermoplastischem Polyurethan, thermoplastischem Elastomer oder glycolmodifiziertem Copolyester (PETG).

10. Faser nach Anspruch 1, die eine Bikomponentenfaser ist mit (1) einer er s-ten Komponente aus einem thermoplastischen hydroxyfunktionalisierten Polyether oder einer Mischung aus einem hydroxyfunktionalisierten Polyether und (2) einer zweiten Komponente aus einem Polyolefin, Polyester, Polyamid, Polysaccharid, modifiziertem Polysaccharid oder natürlich vorkommender Faser oder partikul ärem Füllstoff, thermoplastischem Polyurethan, thermoplastischem Elastomer oder glycolmodifiziertem Copolyester (PETG).

11. Bikomponentenfaser nach Anspruch 10, bei der der hydroxyfunktionalisierte Polyether hergestellt wird durch Umsetzen eines dinucleophilen Monomers mit einem Diglycidylether, einem Diglycidylester oder Epihalogenhydrin.

12. Bikomponentenfaser nach Anspruch 10 oder 11, wobei es sich um eine Side-by-side-Bikomponentenfaser, eine Sheath-core-Bikomponentenfaser, eine Segmented-pie-Bikomponentenfaser oder eine Islands-in-the-sea-Bikomponentenfaser handelt.

13. Bikomponentenfaser nach Anspruch 12, mit einem Kern aus dem therm o-plastischen hydroxyfunktionalisierten Polyether und einem Mantel aus einem thermoplastischen Polymer, das kein hydroxyfunktionalisierter Polyether ist.

14. Bikomponentenfaser nach Anspruch 13, mit einem Mantel aus dem the r-moplastischen hydroxyfunktionalisierten Polyether und einem Kern aus einem thermoplastischen Polymer, das kein hydroxyfunktionalisierter Polyether oder P o-lyester ist.

15. Bikomponentenfaser nach Anspruch 11, die einen zylindrischen, kreuzfö r-migen, trilobalen oder bändchartigen Querschnitt hat.

16. Bikomponentenfaser nach Anspruch 11 in Form eines Filtermediums, einer Bindefaser für Glas- oder Kohlenstofffasern, einer Bindefaser in Vliesstoffen aus einem thermoplastischen Polymer, das kein hydroxyfunktionalisierter Polyether oder Polyester ist, oder einer Bindefaser in Vliesstoffen aus Materialien auf Cell u-losebasis oder in Form eines medizinischen Kleidungsstücks.

17. Web- oder Vliesstoff, der die Faser nach Anspruch 11 und, fakultativ, eine Synthese- oder Naturfaser umfasst.

18. Stoff nach Anspruch 17, bei dem die Synthesefaser ein Polyester, ein Pol y-amid, Reyon oder ein Polyolefin ist und die Naturfaser Baumwolle ist.

19. Stoff nach Anspruch 17 in Form eines Kleidungsstücks, eines wasserabsorbierenden Tuchs, eines Filtergewebes, eines Batterietrennelements, eines a n-tistatischen Lappens oder einer wasserabsorbierenden Matte.

20. Faser nach Anspruch 1 aus einer Mischung von:
(a) einem Poly(hydroxyaminoether) mit Grundeinheiten, die repräsentiert werden durch die Formel: wobei A eine Diaminokomponente oder eine Kombination von ve r-schiedenen Aminkomponenten ist; B eine zweiwertige organische Komponente ist, die vorwiegend Hydrocarbylen ist; R Alkyl oder Wasserstoff ist; und n eine ganze Zahl von 5 bis 1000 ist; und
(b) mindestens einem von einem Polyethylenglycol, Poly(ethylenoxid) oder EPE-Blockcopolymer.

21. Faser nach Anspruch 20, bei der der Poly(hydroxyaminoether) das Reaktionsprodukt von einem Diglycidylether von Bisphenol A und Ethanolamin ist.

22. Verfahren zur Herstellung eines Vliesstoffes durch Bilden eines Vlieses aus mindestens einer Faserkomponente und Erwärmen des Vlieses, damit die Fase r-komponenten des Vlieses verkleben, **dadurch gekennzeichnet, dass** mindestens eine Faserkomponente aus einem thermoplastischen hydroxyfunktionalisierten Polyether nach Anspruch 1 besteht.

23. Verfahren nach Anspruch 22, bei dem mindestens eine Faserkomponente aus einem Poly(hydroxyaminoether) besteht, der Grundeinheiten hat, die repr äsentiert werden durch die Formel: wobei A eine Diaminokomponente oder eine Kombination von verschiedenen Aminkomponenten ist; B eine zweiwertige organische Komponente ist, die vorwi e-gend Hydrocarbylen ist; R Alkyl oder Wasserstoff ist; und n eine ganze Zahl gr ö-βer als 10 ist.
